

Jan. 30, 1945.

M. L. WOOD

2,368,339

PROCESS FOR PRODUCING ALUMINUM BRASSES

Filed June 20, 1944



Inventor  
Maurice L. Wood  
By Seymour E. Nichols  
Attorneys

## UNITED STATES PATENT OFFICE

2,368,339

PROCESS FOR PRODUCING ALUMINUM  
BRASSESMaurice L. Wood, Waterbury, Conn., assignor to  
Chase Brass & Copper Co. Incorporated, Wa-  
terbury, Conn., a corporation of Connecticut

Application June 20, 1944, Serial No. 541,240

1 Claim. (Cl. 75--10)

The present invention relates to improvements in process for producing brasses which contain aluminum.

One object of the present invention is to provide an improved process of producing high-quality brass which contains aluminum in addition to the usual copper and zinc, so that products made of such aluminum-brass will possess physical qualities enabling them to withstand severe distortion without developing defects.

With the above and other objects in view, as will appear to those skilled in the art from the present disclosure, this invention includes all features in the said disclosure which are novel over the prior art.

In the description and claims, the various parts and steps are identified by specific terms for convenience, but they are intended to be as generic in their application as the prior art will permit.

In the accompanying drawing forming part of the present disclosure, in which one way of carrying out the invention is shown for illustrative purposes:

Fig. 1 is a schematic view in central vertical section of an electrical induction furnace suitable for carrying out the present invention, and schematically illustrating one stage of the process; and

Fig. 2 is a view similar to Fig. 1 but schematically illustrating a later stage of the process.

Referring to the drawing, the electric induction furnace 10 has an outer metal casing 11 provided with a refractory lining 12 so as to provide a main chamber 13 which is in communication with two depending chambers in the form of loops 14 and 15. The top of the furnace is provided with a charging-door 16, a skimming-door 17, and a pouring-spout 18. All of the construction of the furnace 10 thus far described is of well-known construction. A pipe 19 is screw-threadedly engaged in an opening 20 opening into the interior top-portion 21 of the furnace. Except when molten metal is being poured out of the furnace through the pouring-spout 18, the spout is kept closed by a removable closure-block 22 of asbestos or other suitable material.

In carrying out my process when starting with the furnace empty, sufficient aluminum-containing brass in molten condition is poured into the furnace through the charging-door 16 to fill the loops 14 and 15 and occupy the lower portion of the main chamber 13, and solid pieces of aluminum-brass, which may consist of ingots, or of scrap such, for example, as tube-ends, extrusion-

butts, billet-gates, saw-chips, etc., are also introduced into the furnace through the charging-door 16, or solid pieces of cathode copper, ingot aluminum and slab zinc may be used with or without the pieces of aluminum brass mentioned. With all furnace openings closed by the parts 16, 17 and 22, hydrogen-containing gas is fed through the pipe 19 so as to fill the upper interior 21 of the furnace so as to maintain the hydrogen-containing gas in contact with the surface of the molten brass and in contact with the surfaces of all pieces of solid brass which extend above the surface of the molten brass. The hydrogen-containing gas is introduced under sufficient pressure to maintain the upper interior 21, above the molten brass, filled with it, so that the gas leaks out of all openings and crevices such, for example, as exist around the charging-door 16, the skimming-door 17, and the closure-block 22, although the arrows adjacent the closure-block 22 are the only arrows used to indicate escape of the gas from the furnace. The escaping gas is preferably disposed of by lighting it at the places where it escapes from the furnace so that the escaping gas burns outside of the furnace. The hydrogen-containing gas should be substantially free of oxygen and of sulfur and of any compound containing oxygen or sulfur, such as water vapor, carbon dioxide, carbon monoxide, hydrogen-sulfide. While hydrogen or any suitable hydrocarbon that can be introduced into the furnace to form gas could be used, I find the well-known hydrocarbon gas "propane" to be convenient and economical for the purpose.

Alternating electric current, acting on the induction principle upon the molten brass occupying the closed loops 14 and 15, as is well understood in the art, heats the molten brass in the loops, and by electric action and by convection, causes molten brass from the loops 14 and 15 to be circulated up into the main-body of molten-brass mixture, and part of the latter circulates down into the loops where the heating takes place.

Finally, after all of the brass becomes molten, there is present in the furnace a molten material or mixture or alloy consisting substantially of copper, zinc, aluminum and small particles of aluminum-oxide, with or without any minor percentage of elements such for example, as antimony or arsenic. It is the small particles of aluminum-oxide which are believed to be the cause of the defects in products made of the alloy. During the time that the unmolten scrap was being heated to raise it to the melting tempera-

ture, the hydrogen-containing gas is thus maintained in contact with the surfaces of the solid pieces of brass, as well as with the surface of the molten portion of the brass, and finally, after all of the brass becomes molten, the hydrogen-containing gas continues to be maintained in contact with the surface of the molten brass, and after several minutes, depending upon the amount of brass being melted, and the rate of heat development by the particular furnace used, the temperature of the molten brass rises from its melting-point of about 1750° F. up to about 2300° F. to 2350° F. As the superheating above the melting-point proceeds, and the temperature rises from about 2000° F. up to 2300° F. or above, zinc is vaporized from the brass in increasing substantial amounts, so as to produce a substantial quantity of zinc vapor, which is indicated in Fig. 2 in the form of what may be referred to as a "blanket" of zinc vapor 23, which is in contact with the surface of the superheated molten brass. After the brass has been raised to the neighborhood of 2300° F. for several minutes, the process is complete, and the brass becomes largely freed of the harmful aluminum-oxide particles. The superheated brass is then poured out of the furnace in a usual and well-known way to make products therefrom.

When the zinc starts to volatilize in ample amounts, this fact is evidenced by a change in color of the gas which issues from the crevices of the furnace and burns, since the zinc vapor, when burning, gives what may be referred to as a characteristic bluish-white light. When the evolution of zinc vapor reaches a high rate, it even issues from the crevices around the charging-door 16.

One particular aluminum-brass upon which my improved process is used is that which has a nominal composition of 76% copper, 2% aluminum and 22% zinc, although aluminum-brasses in which the copper ranges from 70% to 90%, the aluminum from  $\frac{1}{2}\%$  to 3%, and zinc the balance, may also be treated by my process. The evolution of zinc vapor from the zinc content of the brass tends to cause a loss thereof of about one-half of one per cent and therefore, in order to get any particular percentage in the final alloy, a one-half per cent extra amount of zinc is added at the beginning to make up for the loss of zinc in the form of zinc vapor.

During the first part of the process, in which the hydrogen-containing gas is maintained in contact with the surface or surfaces of the molten and non-molten parts of the metal, from the time any of the metal reaches a temperature of about 1000° F. or more, elemental hydrogen from the hydrogen-containing gas, whether present originally as elemental hydrogen or produced as a result of the well-known cracking by heat of hydrocarbon present originally, is absorbed or dissolved in the metal in the form of atomic hydrogen, whether the metal be in molten or in non-molten condition, the rate of absorption and depth of penetration increasing with the temperature of the metal. But it takes place at a higher rate where the metal is in molten condition, not only because the molten metal is ordinarily of a higher temperature than the unmolten metal, but also owing to the stirring action which occurs, particularly the efficient stirring action brought about by the electric action upon the heated loops of molten metal 14 and 15, as previously mentioned. Thus, hydrogen absorbed into the metal has opportunity to chemi-

cally act upon small particles of aluminum-oxide and reduce them to aluminum, thus removing the oxygen from them and joining it to the hydrogen, which then bubbles up through the metal and out above its surface and mixes with the hydrogen-containing gas in the upper portion of the chamber and gradually works its way out through the crevices surrounding the various closure portions of the furnace, as previously described. After the temperature has passed to about 2000° F. and the zinc vapor starts to vaporize in sufficient amount to form the blanket of zinc vapor 23, then hydrogen ceases to enter the metal through its surface, and such hydrogen as remains dissolved in the metal and is in excess and not needed to reduce aluminum-oxide particles, is now caused, as a result of the vaporization of the zinc and formation of the zinc blanket, to pass upward out of the surface of the molten metal and up through the blanket of zinc vapor and mixes with the hydrogen-containing gas above the zinc vapor. Of course, when the evolution of zinc vapor takes place at a very high rate, the depth of the blanket of zinc vapor becomes very deep, in fact, it may extend up so far as to substantially occupy most of the interior space in the furnace, so that, at such a stage, there may be very little hydrogen-containing gas in the furnace, this being evidenced, as previously described, by the burning of bluish-white flames from all crevices of the upper portion of the furnace. And while the zinc vapor at and near the surface of molten metal, will be substantially free from hydrogen-containing gas, except such hydrogen as is evolved from the molten metal, up near the top of the furnace there is a mixture of zinc vapor and hydrogen-containing gas in which the latter is of greater percentage, the higher the position in the furnace that is considered. If no efficient stirring action were to take place, as is accomplished by the loops 14 and 15 as heretofore described, then the first stage of the process would take longer, in order to permit the thorough penetration and mixing of the hydrogen through the molten metal.

When aluminum-containing brass is made in accordance with my process, even where scrap metal is employed to form all of the aluminum-brass mixture, the resultant quality of the metal is so high that the metal when formed into various products, particularly tubes, withstands physical tests indicating its high quality. Thus, one of the most serious troubles encountered is where tubes are made of aluminum-brass, and when such tubes are given what is known as a "flattening test," which consists in completely flattening a portion of tube, unless the metal is of high quality and free from an undue amount of aluminum-oxide particles, surface cracks will appear at the most severely-stressed portions of such flattened tube-portions. Tubes made from metal produced in accordance with my process, however, even from scrap metal, successfully withstand this flattening test without the development of surface cracks.

The invention may be carried out in other specific ways than those herein set forth without departing from the spirit and essential characteristics of the invention, and the present embodiments are, therefore, to be considered in all respects as illustrative and not restrictive, and all changes coming within the meaning and equivalency range of the appended claim is intended to be embraced therein.

I claim:

The process of producing high-quality brasses containing aluminum in addition to the usual copper and zinc contents, the said process comprising: providing an electrically-heated furnace having a melting-chamber and a vent-opening leading outwardly from an upper portion of the said melting-chamber; charging into the lower portion of the melting-chamber of the said furnace, copper, zinc, and aluminum containing aluminum-oxide; supplying into an upper portion of the melting-chamber of the said furnace above the said charge, a hydrogen-containing reducing-gas which is substantially free of sulphur, oxygen and water vapor; electrically energizing the said furnace to effect the melting of the said metals in the melting-chamber thereof while the said reducing gas is present in the said melting-chamber to cause the absorption of hydrogen into the said metals; subsequently raising the temperature of the metals to a point sufficiently above

5 the melting point of the metal mixture to cause the vaporization of sufficient of the zinc to provide a blanket of zinc-vapor directly over the now-super-heated molten metals and maintaining such condition for a sufficient length of time to substantially free the super-heated molten metals of the remaining previously absorbed hydrogen; and maintaining the pressure of the said reducing gas in the melting-chamber of the said furnace at a point sufficiently high to cause an excess thereof to flow outwardly through the vent opening of the furnace during the period of the superheating of the molten metals, to thereby 10 scavenge out from the melting-chamber of the furnace gases and the water vapor which results from the union of hydrogen from the said reducing gas with oxygen derived from the reduction of aluminum-oxide and other oxides originally present in the metals introduced into the furnace.

20

MAURICE L. WOOD.